

Dec. 29, 1964

N. R. HARPSTER

3,163,526

AGE-HARDENABLE AUSTENITIC IRON BASE HIGH TEMPERATURE ALLOYS

Filed March 6, 1963

2 Sheets-Sheet 1



Fig. 1

INVENTOR  
Norman R. Harpster

BY *Weiff, Mackay & Burden*

HIS ATTORNEYS

Dec. 29, 1964

N. R. HARPSTER

3,163,526

AGE-HARDENABLE AUSTENITIC IRON BASE HIGH TEMPERATURE ALLOYS

Filed March 6, 1963

2 Sheets-Sheet 2



Fig. 2

INVENTOR  
Norman R. Harpster

BY *Weil, Mackay & Anderson*

HIS ATTORNEYS

1

3,163,526

AGE-HARDENABLE AUSTENITIC IRON BASE  
HIGH TEMPERATURE ALLOYS

Norman R. Harpster, Canonsburg, Pa., assignor to Universal-Cyclops Steel Corporation, Bridgeville, Pa., a corporation of Pennsylvania

Filed Mar. 6, 1963, Ser. No. 263,312  
8 Claims. (Cl. 75—128)

The present invention relates to austenitic iron base alloys which can be hardened by solution and aging treatments and which are substantially non-magnetic and possess relatively high room temperature properties in combination with satisfactory strength characteristics at elevated temperatures.

This application is a continuation-in-part of application Serial No. 827,157, filed July 15, 1959.

Materials for high temperature applications quite frequently must possess relatively high room temperature properties in combination with good strength properties at elevated temperatures. Several of the so-called super alloys have this desired combination of properties but are relatively expensive. The commonly available austenitic stainless steels possess satisfactory high temperature properties for many applications, but have strength properties at room temperature appreciably below those desired. For some applications, the ordinary austenitic stainless grades have been successfully used by employing cold or hot-cold work to increase room temperature strength. While this method of increasing room temperature properties is satisfactory for some applications, it has many limitations; for example, where forging or welding is employed in fabrication. In such cases, it is not possible to use material initially received in such condition and, therefore, it has been customary to use, for such applications, the more expensive super alloys which can be hardened by heat treatment. A definite need exists for an inexpensive age-hardening austenitic alloy having a combination of good room temperature and elevated temperature properties.

In many applications where both good room temperature and elevated temperature properties are necessary, it is also necessary that the alloy be substantially non-magnetic. This is particularly important in critical magnetic and electrical equipment which should not be magnetically affected by the materials used in nearby structures or tools. A specific application of this type is retainer rings used for supporting large motors. A number of non-magnetic non-ferrous metals super alloys and stainless steels are available for such applications, but the strength and other mechanical properties of such materials are frequently inadequate or fabrication is difficult, or the alloys are too expensive for consideration.

I have found that the desirable attributes indicated above, namely, age-hardenability, high room temperature physical properties, high strength at elevated temperatures, and low permeability, can be obtained in a carbon-manganese-chromium-nickel-vanadium steel by maintaining the various elements mentioned within certain relatively narrow ranges. I have also found that the alloys which I provide remain substantially non-magnetic irrespective of the amount of cold work to which they are subjected and that cold working does not materially modify the age-hardening characteristics. In addition to possessing the above-specified attributes, the alloys of my invention are corrosion resistant and inexpensive to produce since they contain a minimum of high cost alloying elements and can be made by any of the well-known melting practices. Also, the alloys of my invention may be readily hot worked or, if desired for certain types of applications, cold worked without encountering any great difficulty.

FIGURE 1 is a graphical representation of the effect

2

of carbon on the tensile properties of an austenitic iron base alloy in the solution treated and aged condition at room temperature; and

FIGURE 2 is a graphical representation of the effect of vanadium on the tensile properties of an austenitic iron base alloy in the solution treated and aged condition at room temperature.

The alloys of my invention possessing the properties indicated above fall within the following composition ranges:

|            | Percent   |
|------------|-----------|
| Carbon     | 0.35—0.60 |
| Manganese  | 8.0—12.0  |
| Silicon    | 1.0 max.  |
| Chromium   | 6.0—10.0  |
| Nickel     | 4.0—8.0   |
| Vanadium   | 1.1—1.8   |
| Sulphur    | .03 max.  |
| Phosphorus | .05 max.  |
| Iron       | Balance   |

In the alloys of my invention, the austenitic structure is provided by the manganese and nickel and the two, therefore, should be used in such amounts as to assure an austenitic structure, but they also should be maintained within approximately the limits stated above in order to provide adequate non-magnetic properties. When manganese, nickel and other elements mentioned above are maintained within approximately the limits stated, the maximum permeability of the alloys will be approximately 1.2 or less when tested at either 100 or 200 oersteds and will retain their low permeability when subjected to cold working. Vanadium, of course, has an effect on ductility at elevated temperatures and on oxidation resistance and it is, therefore, necessary that the vanadium be kept sufficiently low to avoid either of these adverse effects. Chromium, of course, has a desirable effect on corrosion and oxidation resistance. Therefore, the chromium content should be maintained within the ranges specified in order to achieve adequate corrosion or oxidation resistance and, at the same time, to accomplish the desired precipitation hardening.

While I have specified that the carbon content should be between 0.35 and 0.60% and have not specified the presence of nitrogen, some nitrogen may be present and may be deliberately added during manufacture in order to partially replace or augment the carbon without any material deleterious effect upon the desired properties.

While the broader composition ranges specified above will provide alloys having the above-mentioned properties, a preferred composition range is as follows:

|            | Percent   |
|------------|-----------|
| Carbon     | 0.45—0.60 |
| Manganese  | 8.0—10.0  |
| Silicon    | 1.0 max.  |
| Chromium   | 6.75—8.25 |
| Nickel     | 7.0—8.0   |
| Vanadium   | 1.35—1.65 |
| Sulphur    | .03 max.  |
| Phosphorus | .05 max.  |
| Iron       | Balance   |

A typical alloy embodying my invention is as follows:

|            | Percent |
|------------|---------|
| Carbon     | 0.53    |
| Manganese  | 9.0     |
| Silicon    | 0.50    |
| Chromium   | 7.50    |
| Nickel     | 7.50    |
| Vanadium   | 1.50    |
| Sulphur    | .01     |
| Phosphorus | .035    |
| Iron       | Balance |

As stated above, the alloys of my invention are substantially non-magnetic having a maximum permeability of approximately 1.2. In general, the alloys of this invention will have a permeability less than 1.1. For example, one alloy embodying my invention had a perme-

4  
Samples of alloys embodying my invention were also subjected to similar solution treatments and age-hardened at various temperatures and the tensile properties determined. The various treatments and the tensile properties obtained are set forth below in Table II.

Table II

| Aging Treatment                                                       | 0.02% Yield Strength, p.s.i. | 0.2% Yield Strength, p.s.i. | Ultimate Strength, p.s.i. | Elong., percent | Red. of Area, percent |
|-----------------------------------------------------------------------|------------------------------|-----------------------------|---------------------------|-----------------|-----------------------|
| Solution Treatment: 2,000° F., 1 Hour, Water: 1,300° F., 4 Hours, Air | 69,500                       | 88,000                      | 145,000                   | 33.3            | 51.1                  |
| Solution Treatment: 2,050° F., 1 Hour, Water: 1,300° F., 4 Hours, Air | 96,500                       | 115,500                     | 160,000                   | 25.0            | 50.7                  |
| Solution Treatment: 2,100° F., 1 Hour, Water: 1,300° F., 4 Hours, Air | 139,000                      | 165,000                     | 190,500                   | 9.1             | 18.8                  |
| Solution Treatment: 2,150° F., 1 Hour, Water: None                    | 53,000                       | 59,500                      | 124,500                   | 62.7            | 70.7                  |
| 1,100° F., 16 Hours, Air                                              | 123,500                      | 139,000                     | 163,500                   | 18.3            | 24.3                  |
| 1,200° F., 4 Hours, Air                                               | 115,500                      | 127,500                     | 159,500                   | 30.7            | 33.7                  |
| 1,200° F., 16 Hours, Air                                              | 128,500                      | 157,500                     | 176,500                   | 11.4            | 15.1                  |
| 1,300° F., 4 Hours, Air                                               | 147,000                      | 174,500                     | 199,000                   | 5.9             | 12.3                  |
| 1,300° F., 16 Hours, Air                                              | 140,000                      | 168,000                     | 196,500                   | 7.7             | 11.4                  |
| 1,400° F., 4 Hours, Air                                               | 127,500                      | 154,500                     | 189,000                   | 9.3             | 16.0                  |
| 1,400° F., 16 Hours, Air                                              | 111,500                      | 139,000                     | 178,500                   | 12.7            | 21.1                  |

ability of 1.008 when tested at 50 oersteds and 1.009 when tested at 100 oersteds and at 200 oersteds. The alloy tested had been solution-treated at 2150° F. for one hour, water-quenched, aged for 16 hours at 1300° F. and air-cooled. Another alloy embodying my invention showed a permeability of 1.001 when tested at 100 oersteds and also when tested at 200 oersteds. This alloy had been subjected to the same heat treatment as that just stated. The magnetic characteristics of this alloy were also determined after it had been subjected to cold reductions of 10%, 20%, 30% and 40% and it was found that at each stage of the reduction, the alloy had a permeability of less than 1.002 when tested at 100 oersteds and also when tested at 200 oersteds. This indicates that the composition is quite stable in regard to magnetic characteristics.

In order to determine the response to age-hardening of hot rolled plates embodying my invention, samples were solution treated for one hour at 2000° F., 2100° F., 2150° F. and 2200° F. and water-quenched and then age-hardened at various temperatures for 16 hours and then air-quenched. The Rockwell C hardness values obtained are set forth below in Table I.

Table I

| Heat Treatment           | Rockwell C Hardness             |           |           |           |
|--------------------------|---------------------------------|-----------|-----------|-----------|
|                          | Solution Treatment <sup>1</sup> |           |           |           |
|                          | 2,000° F.                       | 2,100° F. | 2,150° F. | 2,200° F. |
| 1,100° F., 16 Hours, Air | 31.5                            | 32.5      | 35.5      | 35.5      |
| 1,200° F., 16 Hours, Air | 37.0                            | 38.5      | 41.0      | 41.5      |
| 1,300° F., 16 Hours, Air | 36.5                            | 41.5      | 43.5      | 44.5      |
| 1,400° F., 16 Hours, Air | 33.5                            | 40.0      | 43.5      | 43.0      |
| 1,500° F., 16 Hours, Air | 24.5                            | 33.0      | 36.0      | 38.5      |
| 1,600° F., 16 Hours, Air | 20.0                            | 25.0      | 29.5      | 33.0      |
| No Heat Treatment        | 2.97                            | 2.90      | 2.93      | 2.92      |

<sup>1</sup> All samples were treated for 1 hour at indicated temperature and water quenched.

<sup>2</sup> B scale.

35 In addition to the above-mentioned tests, the effects of cold reduction on the alloys of my invention were determined. Hot rolled plates were first solution treated for one hour at 2150° F. and water-quenched. Some of the samples were subjected to cold reduction, the reductions being 10%, 20%, 30% and 40%. Some of the samples were then aged by heating for various times at various temperatures and air-quenched. The Rockwell C hardness values determined for these samples are set forth in Table III.

Table III

| Aging Treatment          | Rockwell C Hardness         |      |      |      |      |
|--------------------------|-----------------------------|------|------|------|------|
|                          | Cold Reduction <sup>1</sup> |      |      |      |      |
|                          | None                        | 10%  | 20%  | 30%  | 40%  |
| None                     | 23.5                        | 31.5 | 41.0 | 43.5 |      |
| 900° F., 4 Hours, Air    | 24.5                        | 33.0 | 40.0 | 43.0 |      |
| 900° F., 16 Hours, Air   | 25.0                        | 34.0 | 43.0 | 46.0 |      |
| 1,000° F., 4 Hours, Air  | 27.0                        | 35.5 | 43.0 | 46.0 |      |
| 1,000° F., 16 Hours, Air | 29.5                        | 36.0 | 45.5 | 47.5 |      |
| 1,100° F., 4 Hours, Air  | 30.5                        | 39.5 | 45.0 | 47.0 |      |
| 1,100° F., 16 Hours, Air | 35.5                        | 37.0 | 43.5 | 47.0 | 50.0 |
| 1,200° F., 4 Hours, Air  | 38.0                        | 37.5 | 43.5 | 46.0 | 48.0 |
| 1,200° F., 16 Hours, Air | 41.0                        | 45.0 | 46.0 | 47.0 | 48.5 |
| 1,300° F., 4 Hours, Air  | 43.5                        | 45.5 | 45.5 | 46.5 | 46.0 |
| 1,300° F., 16 Hours, Air | 45.5                        | 45.0 | 45.5 | 44.5 | 43.0 |
| 1,400° F., 4 Hours, Air  | 42.0                        | 42.0 | 43.0 | 42.0 | 39.0 |
| 1,400° F., 16 Hours, Air | 43.5                        | 42.0 | 43.0 | 39.0 | 35.0 |
| 1,500° F., 4 Hours, Air  | 38.0                        | 40.0 | 38.0 | 38.0 | 35.0 |
| 1,500° F., 16 Hours, Air | 36.0                        | 36.5 | 36.5 | 31.5 | 29.5 |
| 1,600° F., 4 Hours, Air  | 36.5                        | 36.5 | 36.0 | 32.0 | 29.0 |
| 1,600° F., 16 Hours, Air | 32.0                        | 31.5 | 27.5 |      |      |

<sup>1</sup> Hot rolled flats (1½" x 1½") were solution treated for 1 hour at 2,150° F. and water quenched prior to indicated percent cold reduction.

Some of such samples were tested to determine the tensile properties. The treatments to which the material was subjected and the tensile values obtained are set forth below in Table IV.

Table IV

| Aging Treatment                                         | 0.02% Yield Strength, p.s.i. | 0.2% Yield Strength, p.s.i. | Ultimate Strength, p.s.i. | Elong., percent | Red. of Area, percent |
|---------------------------------------------------------|------------------------------|-----------------------------|---------------------------|-----------------|-----------------------|
| Condition: Solution Treated (2,150° F., 1 Hour, Water): |                              |                             |                           |                 |                       |
| None                                                    | 53,000                       | 59,500                      | 24,500                    | 62.7            | 70.7                  |
| 1,200° F., 16 Hours, Air                                | 128,500                      | 157,500                     | 176,500                   | 11.4            | 15.1                  |
| Condition: Solution Treated Plus Cold Reduced 10%:      |                              |                             |                           |                 |                       |
| None                                                    | 77,000                       | 93,000                      | 135,500                   | 50.3            | 65.0                  |
| 1,200° F., 16 Hours, Air                                | 145,500                      | 169,500                     | 192,500                   | 10.8            | 16.7                  |
| Condition: Solution Treated Plus Cold Reduced 20%:      |                              |                             |                           |                 |                       |
| None                                                    | 96,500                       | 123,000                     | 150,000                   | 31.8            | 61.3                  |
| 1,200° F., 16 Hours, Air                                | 144,500                      | 178,500                     | 201,000                   | 4.3             | 8.4                   |
| Condition: Solution Treated Plus Cold Reduced 30%:      |                              |                             |                           |                 |                       |
| None                                                    | 108,500                      | 149,500                     | 170,000                   | 19.8            | 54.0                  |
| 1,200° F., 16 Hours, Air                                | 159,000                      | 188,500                     | 210,500                   | 1.9             | 7.4                   |
| Condition: Solution Treated Plus Cold Reduced 40%:      |                              |                             |                           |                 |                       |
| None                                                    | 120,500                      | 166,500                     | 194,000                   | 14.5            | 49.4                  |
| 1,200° F., 16 Hours, Air                                | 138,500                      | 188,000                     | 218,000                   | 2.5             | 5.6                   |

Forged rings approximately 14 $\frac{1}{8}$ " O.D. by 12 $\frac{1}{8}$ " I.D. were made and subjected to solution and aging treatments and the tensile properties of transverse specimens thereof determined. The treatments and tensile properties are set forth below in Table V.

Table V

| Aging Treatment                                           | 0.02% Yield Strength, p.s.i. | 0.2% Yield Strength, p.s.i. | Ultimate Strength, p.s.i. | Elong., percent | Red. of Area, percent |
|-----------------------------------------------------------|------------------------------|-----------------------------|---------------------------|-----------------|-----------------------|
| Solution Treatment: 2,050° F., $\frac{1}{2}$ Hour, Water: |                              |                             |                           |                 |                       |
| 1,200° F., 4 Hours, Air                                   | 89,500                       | 103,500                     | 146,500                   | 39.6            | 41.8                  |
| 1,300° F., 4 Hours, Air                                   | 117,500                      | 141,000                     | 172,500                   | 18.0            | 32.2                  |
| Solution Treatment: 2,100° F., $\frac{1}{2}$ Hour, Water: |                              |                             |                           |                 |                       |
| 1,200° F., 4 Hours, Air                                   | 110,000                      | 123,500                     | 160,000                   | 27.7            | 28.8                  |
| 1,300° F., 4 Hours, Air                                   | 116,500                      | 151,500                     | 186,000                   | 14.2            | 25.0                  |
| Solution Treatment: 2,150° F., $\frac{1}{2}$ Hour, Water: |                              |                             |                           |                 |                       |
| 1,200° F., 4 Hours, Air                                   | 116,500                      | 134,000                     | 163,000                   | 21.1            | 23.6                  |
| 1,300° F., 4 Hours, Air                                   | 127,000                      | 160,000                     | 191,500                   | 10.4            | 16.3                  |

As stated above, the alloys of my invention have good elevated temperature properties in addition to the other properties specifically mentioned. This is shown by the values set forth below in Table VI. The alloy tested was in the form of hot rolled flats previously subjected to heat treatment at 2100° F. for  $\frac{1}{2}$  hour, water quenched, aged at 1300° F. for 4 hours and then air quenched.

Table VI

| Test Temperature (° F.) | 0.2% Yield Strength (p.s.i.) | Ultimate Strength (p.s.i.) | Elongation (percent) | Reduction of Area (percent) |
|-------------------------|------------------------------|----------------------------|----------------------|-----------------------------|
| Room                    | 160,000                      | 182,500                    | 7.6                  | 14.3                        |
| 400                     | 144,000                      | 167,500                    | 8.1                  | 15.0                        |
| 800                     | 118,000                      | 133,000                    | 11.2                 | 30.2                        |
| 1,000                   | 113,500                      | 122,500                    | 6.4                  | 33.3                        |
| 1,200                   | 90,000                       | 103,000                    | 2.2                  | 8.4                         |
| 1,300                   | 87,000                       | 95,000                     | 3.8                  | 9.0                         |
| 1,400                   | 67,500                       | 72,500                     | 3.0                  | 9.1                         |

It will be seen from Tables I to VI, inclusive, and the information set forth above in regard to magnetic properties that alloys embodying my invention possess the desirable properties mentioned heretofore and it also will be apparent that such alloys can be produced relatively inexpensively.

The superior tensile properties of an alloy having my composition as compared to those of other alloys having the same elements in amounts outside the critical ranges in the alloy of my invention is particularly illustrated by FIGURES 1 and 2. FIGURE 1 shows the results obtained from tests carried out at room temperature on an alloy having the manganese, silicon, chromium, nickel and vanadium within the respective ranges of my composition and in which the amount of carbon was varied from below 0.35% to above 0.60%, the minimum and maximum, respectively, for the alloy of my invention. Each of the alloys was subjected to the same solution treat-

ment and aging prior to testing. As illustrated, an alloy having less than about 0.35% carbon has relatively poor strength properties and relatively high ductility while an alloy having more than about 0.60% carbon exhibits a relatively small increase in strength with a substantial de-

25

crease in ductility as the amount of carbon increases. It is apparent from the curves shown in FIGURE 1 that an alloy having 0.35-0.60% carbon has both good strength and good ductility; whereas less than 0.35% carbon causes a significant decrease in strength and more than 0.60% carbon results in a decrease in ductility without an appreciable increase in strength.

FIGURE 2 shows the results obtained from tests carried out at room temperature on an alloy having the carbon, manganese, silicon, chromium and nickel within the respective ranges of my alloy and in which the amount of vanadium was varied from below 1.1% to above 1.8%, the respective minimum and maximum for the alloy of my invention. Prior to testing, each of the alloys was solution treated and aged in the same manner. The curves of FIGURE 2 show that an alloy having less than about 1.1% vanadium has relatively poor strength characteristics and that the decrease in ductility is relatively small between 1.1 and 1.8% vanadium. If more than about 1.8% vanadium is added to the alloy no increase in either ductility or strength is obtained and, hence, more than 1.8% vanadium merely increases the cost of the alloy without any increase in the physical properties thereof. As shown by FIGURE 2, an alloy having 1.1-1.8% vanadium exhibits significantly higher strength properties than an alloy with less than 1.1% vanadium.

Additional tests have been made to determine the effects of several chemistry variations on the tensile properties of my alloy. The different chemistry variations of the five heats which were melted are shown in Table VII. The first two heats, 1 and 2, have compositions which are outside the range of the alloy of my invention and were remelted for comparison purposes. Heats 3, 4 and 5, respectively, have compositions which represent a low, intermediate and high content of the elements in the alloy of my invention.

7  
Table VII

| Heat Number | Alloying Element, Percent |       |      |       |       |      |          |
|-------------|---------------------------|-------|------|-------|-------|------|----------|
|             | C                         | Mn    | Si   | Cr    | Ni    | V    | Fe       |
| 1           | 0.34                      | 6.48  | 0.38 | 7.62  | 11.40 | 1.09 | Balance. |
| 2           | 0.83                      | 6.65  | 0.31 | 4.02  | 11.52 | 3.65 | Do.      |
| 3           | 0.38                      | 8.65  | 0.04 | 6.78  | 4.48  | 1.47 | Do.      |
| 4           | 0.50                      | 10.23 | 0.39 | 7.86  | 5.94  | 1.73 | Do.      |
| 5           | 0.59                      | 11.57 | 0.59 | 10.00 | 7.52  | 1.72 | Do.      |

In order to test the tensile properties and hardness of the product of each heat four blanks were obtained from each heat which were solution treated at 2100° F. for 1/2 hour, water quenched, age-hardened at 1300° F. for 4 hours and air cooled. After heat treatment, the blanks were machined to a tensile specimen having a gauge length of 1" and a gauge diameter of 0.25". Duplicate tensile tests were conducted at room temperature, 75° F., and at an elevated temperature of 1000° F. on blanks from each heat. The tensile properties and hardness values obtained are set forth in Table VIII.

Table VIII

| Heat Number | Test. Temp. (° F.) | 0.02% Yield Strength (p.s.i.) | 0.2% Yield Strength (p.s.i.) | Ultimate Strength (p.s.i.) | Elongation (Percent) | Reduction of Area (Percent) | Hardness  |
|-------------|--------------------|-------------------------------|------------------------------|----------------------------|----------------------|-----------------------------|-----------|
| 1           | 75                 |                               | 54,000                       | 101,000                    | 59.0                 | 72.0                        | (Ra) 55.0 |
|             | 75                 |                               | 57,000                       | 103,500                    | 55.0                 | 71.5                        | 57.0      |
|             | 1,000              | 26,500                        | 35,000                       | 80,500                     | 38.0                 | 45.5                        | 56.5      |
|             | 1,000              | 27,000                        | 38,500                       | 81,000                     | 33.8                 | 45.5                        | 57.0      |
| 2           | 75                 |                               | 116,000                      | 161,500                    | 18.0                 | 42.5                        | (Rc) 37.5 |
|             | 75                 |                               | 114,000                      | 163,000                    | 17.5                 | 43.0                        | 37.0      |
|             | 1,000              | 63,000                        | 88,500                       | 102,000                    | 12.0                 | 43.5                        | 37.0      |
|             | 1,000              | 59,500                        | 89,000                       | 103,000                    | 12.0                 | 38.0                        | 38.0      |
| 3           | 75                 |                               | 123,500                      | 183,500                    | 20.5                 | 20.5                        | 40.0      |
|             | 75                 |                               | 116,500                      | 176,000                    | 21.5                 | 29.5                        | 40.5      |
|             | 1,000              | 59,500                        | 91,500                       | 103,500                    | 10.5                 | 28.0                        | 39.0      |
|             | 1,000              | 67,500                        | 93,000                       | 102,000                    | 11.0                 | 31.0                        | 40.5      |
| 4           | 75                 |                               | 160,000                      | 191,000                    | 14.5                 | 31.5                        | 44.0      |
|             | 75                 |                               | 162,000                      | 191,500                    | 13.5                 | 31.0                        | 44.5      |
|             | 1,000              | 97,000                        | 117,000                      | 126,000                    | 8.0                  | 24.0                        | 44.0      |
|             | 1,000              | 99,500                        | 117,500                      | 126,000                    | 7.5                  | 27.5                        | 44.0      |
| 5           | 75                 |                               | 165,500                      | 191,500                    | 15.0                 | 32.0                        | 44.5      |
|             | 75                 |                               | 164,500                      | 192,500                    | 15.0                 | 32.0                        | 44.5      |
|             | 1,000              | 84,000                        | 116,500                      | 130,000                    | 10.0                 | 32.5                        | 44.0      |
|             | 1,000              | 93,000                        | 114,000                      | 127,000                    | 10.5                 | 33.5                        | 44.3      |

It is apparent from Tables VII and VIII that an iron base carbon-chromium-manganese-nickel-vanadium alloy in which the elements are within the narrow critical ranges which I have specified has highly desirable and unexpected tensile properties and hardness at both room temperature and elevated temperatures.

My invention may be embodied within the scope of appended claims.

I claim:

1. An austenitic iron base alloy consisting essentially of carbon from about 0.35 to about 0.60%, manganese from about 8.0 to about 12.0%, silicon up to about 1.0% max., chromium from about 6.0 to about 10.0%, nickel from about 4.0 to about 8.0%, vanadium from about 1.1 to about 1.8%, sulphur up to about .03% max., phosphorus up to about .05% max., and the balance substantially all iron and incidental impurities, said alloy being characterized by good physical properties at both room temperature and elevated temperatures, low magnetic permeability, good hot and cold working characteristics and good age-hardenability.

2. An alloy as claimed in claim 1 having a maximum permeability of about 1.2.

3. An austenitic iron base alloy consisting essentially of carbon from about 0.45 to about 0.60%, manganese from about 8.0 to about 10.0%, silicon up to about 1.0% max., chromium from 6.75 to about 8.25%, nickel from about 7.0 to 8.0%, vanadium from about 1.35 to about 1.65%, sulphur up to about .03% max., phosphorus up to about .05% max., and the balance substantially all iron and incidental impurities, said alloy being characterized by good physical properties at both room temperature and

elevated temperatures, low magnetic permeability, good hot and cold working characteristics and good age-hardenability.

4. An alloy as claimed in claim 3 having a permeability not greater than about 1.2.

5. An austenitic iron base alloy consisting essentially of carbon about 0.53%, manganese about 9.0%, silicon about 0.5%, chromium about 7.5%, nickel about 7.5%, vanadium about 1.5%, sulphur about .01%, phosphorus about .035%, and the balance substantially all iron and incidental impurities, said alloy being characterized by good physical properties at both room temperature and elevated temperatures, low magnetic permeability, good hot and cold working characteristics and good age-hardenability.

6. An alloy as claimed in claim 5 having a permeability not greater than about 1.2.

7. Heat treatment hardened austenitic steel articles having a maximum permeability of about 1.2 and good physical properties at both room temperature and elevated temperatures consisting essentially of carbon from

about 0.35 to about 0.60%, manganese from about 8.0 to about 12.0%, silicon up to about 1.0% max., chromium from 6.0 to about 10.0%, nickel from 4.0 to about 8.0%, vanadium from about 1.1 to about 1.8%, sulphur up to about .03% max., phosphorus up to about .05% max., and the balance substantially all iron and incidental impurities, said steel articles being age-hardened by solution annealing, followed by aging at temperatures between 900° F. and 1600° F.

8. Heat treatment hardened austenitic non-magnetic iron base alloy steel articles having good physical properties at both room temperature and elevated temperatures consisting essentially of carbon from 0.35 to about 0.60%, manganese from about 8.0 to about 12.0%, silicon up to about 1.0% max., chromium from about 6.0 to about 10.0%, nickel from about 4.0 to about 8.0%, vanadium from about 1.1 to about 1.8%, sulphur up to about .03% max., phosphorus up to about .05% max., and the balance substantially all iron and incidental impurities, said steel being age-hardened by solution annealing at temperatures in the range from about 2000° F. to 2200° F., cooled and then age-hardened at temperatures between 900° F. and 1600° F.

55 9. Heat treatment hardened austenitic non-magnetic iron base alloy steel articles having good physical properties at both room temperature and elevated temperatures consisting essentially of carbon from 0.35 to about 0.60%, manganese from about 8.0 to about 12.0%, silicon up to about 1.0% max., chromium from about 6.0 to about 10.0%, nickel from about 4.0 to about 8.0%, vanadium from about 1.1 to about 1.8%, sulphur up to about .03% max., phosphorus up to about .05% max., and the balance substantially all iron and incidental impurities, said steel being age-hardened by solution annealing at temperatures in the range from about 2000° F. to 2200° F., cooled and then age-hardened at temperatures between 900° F. and 1600° F.

#### References Cited in the file of this patent

#### UNITED STATES PATENTS

2,815,280 Clarke \_\_\_\_\_ Dec. 3, 1957  
2,865,740 Heger et al. \_\_\_\_\_ Dec. 23, 1958  
3,062,692 Manganello et al. \_\_\_\_\_ Nov. 6, 1962

#### FOREIGN PATENTS

741,053 Great Britain \_\_\_\_\_ Nov. 23, 1955  
562,401 Canada \_\_\_\_\_ Aug. 26, 1958

UNITED STATES PATENT OFFICE  
CERTIFICATE OF CORRECTION

Patent No. 3,163,526

December 29, 1964

Norman R. Harpster

It is hereby certified that error appears in the above numbered patent requiring correction and that the said Letters Patent should read as corrected below.

Columns 5 and 6, Table IV, under the heading "Ultimate Strength, p.s.i.", line 1 thereof, for "24,500" read  
-- 124,500 --.

Signed and sealed this 4th day of May 1965.

(SEAL)

Attest:

ERNEST W. SWIDER  
Attesting Officer

EDWARD J. BRENNER  
Commissioner of Patents